

## UNITED STATES PATENT OFFICE

1,998,767

## CYLINDER OIL

Frederick H. MacLaren, Calumet City, and George F. Bowers, Chicago, Ill., assignors to Standard Oil Company, Chicago, Ill., a corporation of Indiana

No Drawing. Application April 4, 1932,  
Serial No. 603,226

7 Claims. (Cl. 87—9)

This invention relates to lubricants for valves or other mechanical parts that are exposed to steam, i. e., to cylinder oils and the like.

The object of the invention is to provide a lubricant which will withstand severe operating conditions, which will maintain a continuous resistant lubricating film on and between the metal surfaces to be lubricated without "gumming", and which will provide superior lubrication with less oil consumption than has heretofore been possible.

In a common type of lubricator, cylinder oils are forced by a hydrostatic head through an orifice (0.070 in. diameter) into a column of condensed steam, and the emulsion thus formed lubricates the cylinder walls, valves, etc. It is highly desirable that the drops of oil be of small and uniform size so that constant and effective lubrication may be accomplished with a minimum consumption of oil. Refined oils tend to have large drop sizes but refinement is necessary to obtain other essential properties. Heretofore special chemicals or agents, such as lead oleate, sperm oil, etc., have been used to lower and regulate drop size. An object of our invention is to avoid the use of such special chemicals or agents, and at the same time to obtain a drop size of about .065 cc. which has been found desirable in practice.

A further object is to provide a lubricant which will increase the efficiency of the steam engines or compressors in which it is used. A further object is to provide a lubricant of this type at less cost than has heretofore been possible. Other objects will be apparent from the following detailed description.

We have discovered that when a heavy steam refined oil is compounded with small amounts of hydrogenated fats, startling results are obtained. Previous experiments showed that No. 1 lard oil was superior as a compounding agent to prime lard oil, acidless tallow oil, degras, etc. We have now discovered that hydrogenated fat, which preferably contains a small amount of free fatty acid, increases to a marked extent the desirable properties of these prior oils and in addition, it accomplishes a new result: it stabilizes the drop size of the lubricant, and in the lubricator above described it gives a drop size of 0.065 cc. We dispense entirely with added stabilizers, and at the same time we obtain a greater uniformity of drop size than has been heretofore known in lubricants of this type.

Our invention may be applied to lubricants of the "invert emulsion" type which contain alumini-

num stearate or equivalent soaps, asphaltic materials, etc., and which thereby cause the formation of a water-in-oil emulsion. The invention is also applicable to lubricants which contain no emulsifying agents. In either case the adhesive and lubricating qualities of the oil are increased and the drop size accurately controlled.

The following formulae will exemplify preferred embodiments of the invention:

| Example A                              | Per cent |
|----------------------------------------|----------|
| Mid-Continent steam refined            | 91.5     |
| Hydrogenated fats (.5 free fatty acid) | 8.5      |

| Example B                               | Per cent |
|-----------------------------------------|----------|
| Mid-Continent steam refined             | 90.7     |
| Aluminum stearate                       | 0.8      |
| Hydrogenated fats (.5% free fatty acid) | 8.5      |

| Example C                                   | Per cent |
|---------------------------------------------|----------|
| Mid-Continent steam refined                 | 95.2     |
| Aluminum stearate                           | 0.8      |
| Hydrogenated fish oil (20% free fatty acid) | 4.0      |

| Example D                   | Per cent |
|-----------------------------|----------|
| Mid-Continent steam refined | 93.2     |
| Asphaltic material          | 2.0      |
| Hydrogenated fats           | 4.0      |
| Aluminum stearate           | 0.8      |

The oil in these examples may be described as a heavy steam-refined Mid-Continent lubricating oil having a flash point of about 530° F. and a viscosity at 210° F. of about 175 seconds Saybolt. The flash point and viscosity are not critical and are determined by the particular lubrication problem. Instead of using Mid-Continent steam refined lubricating oils we may use heavy Pennsylvania steam refined oils or equivalent oils from other crudes.

The hydrogenated fats are prepared from mixtures of fish oils, cotton seed oils, rape seed oils, etc. Fish oils are particularly desirable, since they contain largely unsaturated glycerides having 18 carbon atoms (olein and its isomers, some of which are elaidin, iso-olein, and petroselinin). The titre of the hydrogenated acids is usually controlled by suitably proportioning the amounts of cottonseed oil, rape seed oil, etc. which are added to the fish oil, and for the present purpose we prefer to use an oil or fat with a titre of about 42° C. The particular process of hydrogenating these oils is well known (see pages 50 to 55).

372-430 of "Hydrogenation of Organic Substances" by Carleton Ellis, D. Van Nostrand Company, Inc., 250 Fourth Avenue, New York, Third Edition, 1930), and since it forms no part of the present invention it will not be described in detail. The hydrogenated oils are characterized by high saturation and uniformity, and they may be prepared with accurately regulated free fatty acid contents of from 0.5% to 20.0%. We do not limit ourselves to any particular hydrogenated oil, but we prefer to use hydrogenated fish oils.

The asphaltic material is preferably obtained from a cracked petroleum resin because asphalts of this type are characterized by their fluidity at high temperatures. The asphalt in Example D has a melting point of about 135-145° F. and a penetration of about 5-20 at 77° F.

The proportions stated in the above formulae are by way of example only and it may be generally said that the hydrogenated fat content may vary from about 2.0% to 15%, the aluminum stearate may vary from 0 to 2.0% and the asphaltic material from 0 to 5.0%. The effect of hydrogenated fats on heavy steam refined lubricating oils does not depend on any particular proportion within the limits above stated, but depends rather on the compounding of the oil with said hydrogenated fats.

We have described the use of aluminum stearate as an emulsifier for obtaining water-in-oil emulsions, also called "invert emulsions". It should be understood that any emulsifier with this property may be used instead of aluminum stearate, and particularly we may mention calcium stearate and iron stearate. Oleates may be used, but they may be objectionable from the standpoint of gum formation.

The drop size of an oil is determined by discharging the oil upwardly into hot water (about 200° F.) from an orifice about 0.070 in. in diameter under a head of about one or two inches of water, the drops issuing at the rate of about six per minute. Size is computed by dividing volume in cc. by the number of drops. Oils compounded with lard oil give drop size of 0.18 to 0.30 cc.—much too large. By using sperm oil it has been possible to bring the drop size down to .08-.11 cc. but the size varies somewhat from time to time. We have discovered that by compounding these steam refined heavy oils with hydrogenated fats we may obtain a uniform drop size of .065 cc. and that this drop size is the same, for instance, for a heavy paraffin oil as for a mixture of paraffin and Casper steam refined oils of equivalent viscosities.

In the lubrication of compressors, steam engines and similar apparatus it is common practice to supply the oil through a dropper or lubricator, and it is of extreme importance that the drop size be uniform and constant.

The cylinder oils prepared in accordance with the above formulae have been subjected to severe laboratory tests and to tests on compressors and steam engines, particularly in lubricating Corliss valves on steam engines. In en-

gine tests the engine speed was maintained at about 4,000 to 5,000 revolutions per hour and .05 pounds of oil were used per thousand revolutions in all tests. As above described (see Examples A to D) the oils compounded gave perfect lubrication,—at no time was there any noise or undue vibration of the valves, and at the end of three days, when the valves were inspected, there were perfect oil films with no signs of dry spots, no signs of wear, and no signs of the presence of gum on the valve ends. It was not necessary during the tests on these oils to add additional oil or to change the setting of the lubricator. The drop size was uniformly about .065 cc. which insured dependable thorough and constant lubrication.

While we have described in detail preferred embodiments of our invention, it should be understood that we do not limit ourselves to the details or proportions above described except as defined by the following claims which should be construed as broadly as the prior art will permit.

We claim:

1. A composition for lubricating steam cylinders and steam valves which composition consists essentially of a heavy hydrocarbon lubricating oil, about 1% to 10% of a hydrogenated fat, about .5% to 20% of free fatty acid, and a small amount of oil-soluble soap selected from the class consisting of calcium stearate, iron stearate and aluminum stearate, the composition being normally liquid and characterized by a uniformly small drop size when introduced through the orifice of a lubricator into a steam cylinder.

2. The composition covered by claim 1 in which the hydrogenated fat is selected from the class consisting of fish oils, cotton seed oils, rape seed oils and mixtures thereof.

3. The composition of claim 1 which includes a small amount of asphaltic material.

4. A composition for lubricating steam cylinders and steam valves which consists essentially of a heavy steam-refined lubricating oil having a viscosity at 210° F. of the order of 175 seconds Saybolt, and about 1% to 15% of a hydrogenated fat containing about .5% to 20% of free fatty acid, the composition being a liquid having a drop size of about .065 cc. when introduced through an orifice of .07 inch in diameter into water at about 200° F. at the rate of about 6 drops per minute.

5. The composition of claim 4 which includes a small amount of aluminum stearate.

6. The composition of claim 4 which includes a small amount of asphaltic material.

7. A composition for lubricating steam cylinders and steam valves which consists essentially of about 93.2% of heavy Mid-Continent steam-refined lubricating oil having a viscosity at 210° F. of about 175 seconds Saybolt, about 2% of asphaltic material, about 4% of hydrogenated fats, and about .8% of aluminum stearate.

FREDERICK H. MACLAREN,  
GEORGE F. BOWERS.